

# United States Patent [19]

Kishida et al.

[11] Patent Number: 4,992,414

[45] Date of Patent: Feb. 12, 1991

[54] THERMAL TRANSFER RECEIVING SHEET

[75] Inventors: Seiichiro Kishida; Toshiaki Aono; Tetsu Kamosaki, all of Kanagawa, Japan

[73] Assignee: Fuji Photo Film Co., Ltd., Kanagawa, Japan

[21] Appl. No.: 413,817

[22] Filed: Sep. 28, 1989

[30] Foreign Application Priority Data

Sep. 30, 1988 [JP] Japan ..... 63-247218

[51] Int. Cl.<sup>5</sup> ..... B41M 5/035; B41M 5/26

[52] U.S. Cl. ..... 503/227; 8/471; 428/195; 428/342; 428/478.8; 428/513; 428/913; 428/914

[58] Field of Search ..... 8/471; 428/195, 478.2, 428/478.8, 513, 913, 914, 341, 342; 503/227

[56]

References Cited

U.S. PATENT DOCUMENTS

4,720,480 1/1988 Ito et al. ..... 503/227  
4,774,224 9/1988 Campbell ..... 503/227

FOREIGN PATENT DOCUMENTS

61-295085 12/1986 Japan ..... 503/227

Primary Examiner—Bruce H. Hess

Attorney, Agent, or Firm—Sughrue, Mion, Zinn, Macpeak & Seas

[57]

ABSTRACT

A thermal transfer receiving sheet adapted to receiving a dye from a thermal transfer sheet containing a dye capable of being sublimed or rendered mobile by heat, wherein said thermal receiving sheet comprises at least one receiving layer for receiving dye provided on a base sheet, and said base sheet comprises a support having at least one hydrophilic binder provided on the support between the support and the receiving layer.

3 Claims, No Drawings

## THERMAL TRANSFER RECEIVING SHEET

## FIELD OF THE INVENTION

This invention concerns thermal transfer receiving sheets which are used in combination with thermal transfer sheets which have dye donating layers which contain dyes which are sublimed or rendered mobile by heat and, more precisely, the invention concerns thermal transfer receiving sheets with which there is little blurring or fading of the image on ageing after the image has been formed.

## BACKGROUND OF THE INVENTION

Various information processing systems have been developed to meet the demands of the rapid expansion which has taken place in the information industry in recent years, and methods of recording and apparatus compatible with these information processing systems have been developed and adopted. Heat sensitive recording methods are such that the apparatus used is light and compact, there is little noise associated with the apparatus and they have excellent operability and maintenance characteristics and, since they also allow coloring to be achieved easily, these methods are the most widely used.

The heat sensitive transfer recording systems can be broadly classified into two types. In the first type, heat is imagewise applied from the support side to a thermofusible ink which has been coated onto the support and the ink is fused in the form of the pattern in which the heat has been applied and transferred to the recording medium to provide a hard copy. In the second system, heat is applied from the support side in the same way as before to a heat sensitive transfer sheet which has, on a support, a layer which contains a dye which is sublimed or rendered mobile by heat, the dye migrates into the recording medium (receiving sheet) in the form of the pattern in which the heat has been applied and a hard copy is obtained.

The recording media (thermal transfer receiving sheets) used here have a receiving layer comprising a resin which is easily dyed with dyes which receiving layer is coated on, or attached by pressure to, a base sheet such as paper or a PET base.

Among the properties required of the base sheet, it should be capable of forming an image of high density as a result of the transfer and it should provide good image storage properties with no fading of the image even on ageing after the image has been formed.

The composition of the receiving layer can be improved and the diffusibility of the dye can be increased with a view to raising the transfer density.

Furthermore, image fading arises as a result of movement in the receiving layer itself and diffusion of the dye, and if the base sheet has properties which enable the dye to diffuse, it is diffused through the base sheet and image fading occurs. It is clear that fading of the image occurs for this reason especially when polyethylene coated papers are used for the base sheet. Consequently, there is a problem in that fading of the image is liable to occur when resins which provide high dye diffusibility are used with the intention of increasing the transfer density on a polyethylene coated paper.

## SUMMARY OF THE INVENTION

An object of this invention is to provide thermal transfer receiving sheets with which a high transfer

density can be obtained and with which the extent of image fading is slight.

The above and other objects of this invention will be more apparent from the following description.

5 The objects of the invention have been achieved by means of a thermal transfer receiving sheet adapted to receiving a dye from a thermal transfer sheet containing a dye capable of being sublimed or rendered mobile by heat, wherein the thermal receiving sheet comprises at least one receiving layer for receiving dye provided on a base sheet, and the base sheet comprises a support having at least one hydrophilic binder provided on the support between the support and the receiving layer.

Moreover, thermal transfer receiving sheets in which an intermediate layer which is formed using a hydrophilic synthetic resin and/or synthetic resin aqueous emulsion is established on a synthetic paper and the receiving layer is established on this layer have been disclosed in JP-A-61-295085. (The term "JP-A" as used herein signifies an "unexamined published Japanese patent application"). However, the objective in this case is to prevent the occurrence of the disadvantages which arise when a synthetic paper is used as a support, that is to prevent curling during heating and transfer and concave type deformation in the heated parts, and the use of a comparatively large amount (3 to 20 g/m<sup>2</sup>) of a water soluble synthetic resin or synthetic resin aqueous emulsion is required for this purpose. If the amount of synthetic resin aqueous emulsion used is increased in terms of the coated weight or in terms of the preferred ratio for the conjoint use of the water soluble synthetic resin and synthetic resin aqueous emulsion, there is insignificant prevention of image fading with the passage of time on storing, and if the amount of water soluble synthetic resin is increased then curl is liable to increase and problems arise in practice.

This invention is distinguished by the fact that a layer comprising as small an amount as possible of a hydrophilic binder is established in order to reduce the extent of image fading on ageing and to prevent the occurrence of curling, and this is essentially different from the invention disclosed in the aforementioned prior arts.

## DETAILED DESCRIPTION OF THE INVENTION

The invention is described in detail below.

Thus, basically, the thermal transfer receiving sheets 50 of this invention are constructed with a base sheet, an image receiving layer and a hydrophilic binder layer which is present between the base and the image receiving layer.

Examples of hydrophilic binders which can be used 55 in the hydrophilic binder layer in this invention include vinyl polymers and derivatives thereof, such as polyvinyl alcohol, polyvinylpyrrolidone, poly(vinylpyridium) and cationic modified polyvinyl alcohol (as disclosed, e.g., in JP-A-60-145879, JP-A-60-220750, JP-A-61-143177, JP-A-61-235182, JP-A-61-245183, JP-A-61-237681 and JP-A-61-261089 incorporated herein by reference), polymers which have an acrylic group, such as polyacrylamide, polydimethylacrylamide, polydimethylaminoacrylate, polyacrylate or a salt 60 thereof, acrylic acid/methacrylic acid copolymer or a salt thereof, polymethacrylate or a salt thereof and acrylic acid/vinyl alcohol copolymers or a salt thereof (as disclosed, e.g., in JP-A-60-168651 and JP-A-62-9983

incorporated herein by reference), natural polymers and derivatives thereof, such as starch, oxidized starch, starch acetate, starch amine, carboxyl starch, dialdehyde starch, cationic starch, dextrin, sodium alginate, gum arabic, casein, pullulan, dextran, methylcellulose, ethylcellulose, carboxymethylcellulose, hydroxyethylcellulose and hydroxypropyl cellulose (as disclosed, e.g., in JP-A-59-174382, JP-A-60-262685, JP-A-61-143177, JP-A-61-181679, JP-A-61-193879 and JP-A-61-287782 incorporated herein by reference), synthetic polymers such as polyethylene glycol, polypropylene glycol, polyvinyl methyl ether, maleic acid/vinyl acetate copolymers, maleic acid/N-vinylpyrrolidone copolymers, maleic acid/alkyl vinyl ether copolymers and polyethyleneimine (as disclosed, e.g. in JP-A-61-32787, JP-A-61-237680 and JP-A-61-277483 incorporated herein by reference), and the hydrophilic polymers as disclosed, e.g., in JP-A-56-58869 incorporated herein by reference.

Furthermore, the partially crosslinked hydrophilic polymers known as highly water absorbent polymers, such as starch - polyacrylonitrile hydrolyzate, starch - polyacrylic acid salt crosslinked material, carboxymethylcellulose crosslinked material, ketonized vinylacetate/methyl acrylate copolymer, and poly(sodium acrylate) crosslinked material (for example, as disclosed in "Hi-tech Polymer Materials", page 216, published 1986, Agune Publishing Co. incorporated herein by reference) can be used in the invention.

Among these, hydrophilic binders capable of being crosslinked by hardeners are preferred.

When compared with water soluble synthetic resins and synthetic resin aqueous emulsions, the use of gelatin for the hydrophilic binder has a greater effect on reducing the level of fading and, moreover, since it can be set-dried, there is very little dry tack and this is especially desirable. In practical terms, gelatins and derivatives thereof, such as lime treated gelatin, lime treated gelatin which has been subjected to a calcium removing treatment, acid treated gelatin, phthalated gelatin, acetylated gelatin and succinylated gelatin, for example, and enzyme treated gelatins such as those described in *Bull. Soc. Phot. Japan*, No. 16 p.30 (1966), and gelatin hydrolyzates and enzyme degradation products, can be used for this purpose.

The amount of hydrophilic binder coated is within the range which suppresses fading of the image on ageing, and the use of as small a quantity as possible is preferred from the viewpoint of minimizing the effect on other characteristics such as curl, for example.

In practice, the amount used differs according to the type of hydrophilic binder and the type of base sheet, but of hydrophilic binder and the type of base sheet, but the use of an amount of a hydrophilic binder from 0.1 to 8 g/m<sup>2</sup> is preferred, the use of an amount of from 0.2 to 5 g/m<sup>2</sup> is more preferred, the use of an amount of from 0.4 to 3 g/m<sup>2</sup> is especially preferred, and the use of from an amount of from 0.4 to 2.5 g/m<sup>2</sup> is most preferred.

In general, image fading is seen to improve with coated weights of at least 0.1 g/m<sup>2</sup>, there is a further improvement with coated weights of at least 0.2 g/m<sup>2</sup>, and there is a pronounced improvement with coated weights of at least 0.4 g/m<sup>2</sup>.

Furthermore, a coated weight of not more than 3 g/m<sup>2</sup> is preferred for preventing the occurrence of curl, especially when gelatin is used as the hydrophilic binder.

The hydrophilic binder layer may contain binders other than hydrophilic binders, but large amounts such that the minimizing effect on image fading is lost should not be used. In this invention it is preferred that at least 5 50 wt%, more preferred that at least 70 wt%, and most preferred that at least 90 wt%, of the solid fraction of the hydrophilic binder layer should consist of the hydrophilic binder.

The hydrophilic binder layer can be formed by coating on the support (base sheet) with the addition of coating promoters, viscosity increasing agents, hardeners, surfactants etc.

Examples of the hardener include those described in U.S. Pat. No. 4,678,739 (column 4,), JP-A-59-116655, 15 JP-A-62-245216 and JP-A-61-18942. Specific examples thereof include aldehyde type hardener such as formaldehyde, aziridine type hardener, epoxy type hardener such as



20 vinylsulfone type hardeners such as N,N'-ethylenebis(- vinylsulfonylacetamide)ethane, N-methylol type hardeners such as dimethylol urea, and polymer hardeners such as those described in JP-A-62-234157.

No particular limitation is imposed upon the base sheets used for the thermal transfer receiving sheets of 30 this invention, and any of the known base sheets can be used. In the invention, materials in which the dye has a high diffusibility can also be used as base sheets.

Practical general examples are indicated below. (1) Synthetic Papers (for example polyolefin based and 35 polystyrene based synthetic papers). (2) Paper supports, such as high grade paper, art paper, coated papers, cast coated papers, wall paper, lining paper, synthetic resin or emulsion impregnated papers, synthetic rubber latex impregnated papers, synthetic resin internally added 40 papers, cardboard, cellulose fiber paper and polyolefin coated paper (especially papers which have been covered on both sides). (3) Various plastic films or sheets, such as polyolefin, polyvinyl chloride, polyethylene terephthalate, polystyrene, methacrylate or polycarbonate films or sheets, and films and sheets which have 45 been treated in such a way as to impart white reflecting properties to these plastics.

Furthermore, use can also be made of laminates in which any of the sheets or plates described in (1) to (3) 50 above are combined.

Actual examples of base sheets in which dyes have a high diffusibility include polyolefin based or polystyrene based synthetic papers, polyolefin based or polystyrene based plastic films or sheets and polyolefin coated papers (especially polyethylene coated paper).

Of these, the use of polyolefin coated paper is preferred since it has many advantages in that concave deformation due to heating does not occur during the thermal transfer process, it has excellent whiteness and it exhibits little curl. With polyolefin coated papers, the dyes are highly diffusible in the polyolefin so that fading is liable to occur, but the occurrence of fading can be prevented effectively by means of this invention.

55 Polyolefin coated paper (especially polyethylene coated paper) has been described, for example, on pages 223 to 240 of the Japanese Photographic Society publication entitled "Fundamentals of Photographic Engineering (Silver Salt Photography Edition)" (Published

by Corona, 1979). Polyethylene coated paper consists essentially of a support sheet and a layer of polyethylene which has been coated on the surfaces of the support. The support sheet may consist of materials other than synthetic resins and high grade paper is generally used. The polyethylene coating may be established on the surface of the support sheet (core paper) using any method to attach the polyethylene layer, but such coating is usually achieved using an extrusion method. The polyethylene coating layer may be established on just the side of the support sheet on which the receiving layer is to be established or polyethylene layers may be established on both sides of the base sheet. The type of polyethylene used can be classified by density into high density polyethylene and low density polyethylene, and either type may be used. However, in consideration of the thermal insulating effect during transfer, the use of low density polyethylenes which have a lower thermal conductivity is preferred on the side on which the receiving layer is established.

No particular limitation is imposed upon the thickness of the polyethylene coating, but a thickness of from 5 to 100  $\mu\text{m}$  per side is usually preferred. However, thinner polyethylene coatings (preferably from 5 to 40  $\mu\text{m}$ , more preferably from 5 to 20  $\mu\text{m}$ ) on the receiving layer side are preferred in order to achieve higher transfer densities.

Pigments and fillers such as titanium oxide and ultramarine, for example, can be added to the polyethylene coating to increase whiteness.

Furthermore, the ethylene coated papers may have a thin gelatin layer of from some 0.05 to 0.4  $\text{g}/\text{m}^2$  established on the surface (on the side on which the receiving layer is established and/or on the reverse side). The coated weight of this gelatin layer is included in the coated weight of the hydrophilic binder of this invention.

A dye receiving layer is established as the image receiving part of the thermal transfer receiving sheet. This receiving layer takes in the dye which migrates from the thermal transfer sheet during printing and functions in such a way as to be dyed by the dye, and it preferably has a thickness of from 0.5 to 50  $\mu\text{m}$ , and more preferably of from 1 to 20  $\mu\text{m}$ .

Synthetic resins which can be used for the receiving layer are indicated below.

(a) Those which have Ester Bonds: For example, polyester resins, polyacrylic acid ester resins, polycarbonate resins, polyvinyl acetate resins, styrene acrylate resins and vinyltoluene acrylate resins. Actual examples have been disclosed in JP-A-59-101395, JP-A-63-7971, JP-A-7972, JP-A-63-7973 and JP-A-60-294862. Furthermore, "Vylon 290", "Vylon 200", "Vylon 280", "Vylon 300", "Vylon 103", "Vylon GK-140", and "Vylon 130" made by Toyobo Co., Ltd., and "ATR-2009" and "ATR-2010" made by Kao Corporation, for example, can be used as commercial products.

(b) Those which have Urethane Bonds: For example polyurethane resins.

(c) Those which have Amide Bonds: For example polyamides.

(d) Those which have Urea Bonds: For example urea resins.

(e) Those which have other Highly Polar Bonds: For example, polycaprolactone resins, styrene/maleic anhydride resins, poly(vinyl chloride) resins, polyacrylonitrile resins.

In addition to the synthetic resins described above it is possible to use mixtures or copolymers of these materials. Furthermore, receiving layers can be formed from two or more types of resin which have different properties.

The use of polyester resins or mixtures of resins which at least contain polyester resins is preferred for the receiving layers of this invention.

The receiving layer can be provided by coating a solution obtained by dissolving the above dye receiving polymers (synthetic resins) in an organic solvent on a base sheet followed by drying. Also, it can be provided by coating an emulsion dispersion of the dye receiving polymer in an organic solvent in an aqueous solution of water-soluble polymers, or a latex of the dye receiving polymers dispersed in an aqueous solution of water-soluble polymers on a base sheet followed by drying.

As the above water-soluble polymers, those described for the hydrophilic binders can be used. Among these, polymers capable of being crosslinked by a hardener is preferred, and gelatin and derivatives thereof and polyvinyl alcohol are more preferred.

The receiving layer may be constituted by two or more layers. In this case, the layer near the base sheet may be formed of a dye receiving polymer having a low glass transition point or added with a high boiling point solvent or a thermal solvent so as to increase the solubility to the dye, and thereby the density of the transferred image can be increased. By using, in the outermost

layer, a dye receiving polymer having a higher glass transition point or containing no or a little amount of high boiling point solvents or thermal solvents, sticking or adhesion of the surface of the receiving layer to other materials, retransfer of the transferred image to other materials, and malfunctions such as blocking with the thermal transfer material can be prevented. In the case where the receiving layer has a double-layer structure, the outermost layer preferably has a thickness of from 0.1 to 2  $\mu\text{m}$ , more preferably from 0.2 to 1  $\mu\text{m}$ .

High transfer densities can be obtained in general when resins which have a low glass transition temperature are used, but in this case the extent of image fading on ageing after image formation is pronounced. However, this fading can be greatly reduced in extent by the

incorporation of a hydrophilic binder layer of this invention and so it is possible to obtain both a high transfer density and little fading on storage using resins which have a comparatively low glass transition temperature. The effect of the invention is especially pronounced when resins which have a low glass transition temperature are used in the form of comparatively thin layers.

In this invention, known crosslinking agents can be used to crosslink the receiving layer polymers. Actual examples of crosslinking agents which can be used have been disclosed in JP-A-58-215398 and JP-A-61-199997. The use of isocyanate based crosslinking agents is especially preferred with the polyester resins.

High boiling point organic solvents or thermal solvents can be used as melting point depressants to obtain high transfer densities in this invention.

The high boiling point organic solvents are preferably solvents which are liquid at normal temperature and which do not boil at the heating temperature, and they include esters (for example, phthalate esters, phosphate esters, fatty acid esters), amides (for example aliphatic amides, sulfoamides), ethers, alcohols, paraffins and silicone oils.

Thermal solvents which can be used are compounds which (1) are compatible with dyes, (2) which are solids at normal temperatures but which melt when heated by the thermal head during printing (this may involve mixed melting with other components) and (3) which do not decompose on being heated by the thermal head. The preferred compounds have a melting point of 35° to 250° C., and preferably of from 35° to 200° C., and a value for the ratio (inorganic nature/organic nature) of less than 1.5. Here, inorganic nature and organic nature are factors which provide an indication of the nature of the compound, and this has been described in detail, for example, in "The Realms of Chemistry", vol. 11, page 719, (1957). In practical terms, the compounds disclosed in JP-A-62-136646 can be used for this purpose.

The high boiling point organic solvents and/or thermal solvents can be present individually in the form of a microdispersion in the accepting layer, or they may be present in the form of a suitable mixture with other components such as binders.

The above mentioned high boiling point solvents can also be used to improve slip properties, adhesion resistance, peeling properties and the curl balance, for example.

Furthermore, fillers such as silica, clay, talc, diatomaceous earth, calcium carbonate, calcium sulfate, barium sulfate, aluminum silicate, synthetic zeolites, zinc oxide, lithophane and titanium white, for example, may also be added to the receiving layer or an underlayer.

Release agents can be included in the receiving layer, or a releases agent layer can be established over the receiving layer, in order to improve the peelability of the thermal transfer sheet from the thermal transfer receiving sheet of this invention. Release agents which can be used for this purpose include, for example, solid waxes such as polyethylene wax and amide wax, teflon powder, fluorine based and phosphate ester based surfactants and silicon oils, and the use of silicone oils is especially desirable.

Liquid silicone oils can be used for this purpose but the use of curable oils is preferred. From among the silicone oils, the use of modified silicone oils is preferred. Actual examples include amino modified silicone oils such as KF-393, KF-857, KF-858 and X-22-3680, X-22-3801, epoxy modified silicone oils such as KF-1001, KF-101, KF-103 and X-60-164, catalytically or photocurable silicone oils such as KS-705F-OS (catalytic), KS705F-PS-1 (catalytic), KS720, KS770-PL-3 (catalytic) and KS774-PL-3 all made by Shin-etsu Chemical Co., Ltd. Among these materials the use of the amino modified silicone oils is especially preferred.

The thickness of the release agent layer is from 0.01 to 5  $\mu\text{m}$ , and preferably from 0.05 to 2  $\mu\text{m}$ . The release agent layer may be coated by adding silicone oil to the receiving layer and then curling the silicone oil which subsequently bleeds out of the surface of the receiving layer.

In this invention, further anti-color fading agents can also be included in the receiving layers described above. The anti-color fading agents may be included in the receiving layer by addition to, or by dispersion or dissolution in, the coating composition used for forming the receiving layer. Examples of anti-color fading agents include antioxidants, ultraviolet absorbers and various metal complexes. Examples of antioxidants include chroman based compounds, coumarane based compounds, phenol based compounds (for example hindered phenols), hydroquinone derivatives, hindered

amine derivatives and spiroindane derivatives. The compounds disclosed in JP-A-61-159644 are also effective in this connection.

Examples of ultraviolet absorbers include benzotriazole based compounds (for example, U.S. Pat. No. 3,533,794), 4-thiazolidone based compounds (for example, U.S. Pat. No. 2,252,681), benzophenone based compounds (for example, JP-A-46-2784), and the other compounds disclosed, for example, in JP-A-54-48535, JP-A-62-136641 and JP-A-61-88256. Furthermore, the ultraviolet absorbing polymers disclosed in JP-A-62-260152 are also effective for this purpose.

Examples of metal complexes include the compounds disclosed, for example, in U.S. Pat. No. 4,241,155, columns 3 to 36 of U.S. Pat. No. 4,245,018, columns 3 to 8 of U.S. Pat. No. 4,254,195, JP-A-62-174741, pages 27 to 29 of JP-A-61-88256, JP-A-1-77045 and JP-A-63-199248. Examples of useful anti-color fading agents have been disclosed on pages 125 to 137 of JP-A-62-215272.

The above mentioned antioxidants, ultraviolet absorbers and metal complexes may be used in combinations.

Moreover, fluorescent whiteners can be included in the receiving layers described earlier in this invention. The compounds described, for example, by K. Venkataraman in "The Chemistry of Synthetic Dyes", volume 5, chapter 8, and those disclosed in JP-A-61-143752 can be cited as examples of fluorescent whiteners include stilbene based compounds, coumarin based compounds, biphenyl based compounds, benzoxazolyl based compounds, naphthylimide based compounds, pyrazoline based compounds, carbostyryl based compounds and 2,5-dibenzoxazolylthiophene based compounds. The fluorescent whiteners can be used in combination with anti-color fading agents.

The thermal transfer receiving sheets of this invention may have intermediate layers which do not contain a hydrophilic binder between the base sheet and the receiving layer. However, if an intermediate layer which does not contain a hydrophilic binder such that dyes have a high diffusibility in the layer, it is necessary to provide a hydrophilic binder layer between this intermediate layer and the receiving layer. In cases where the intermediate layer which does not contain hydrophilic binder is such that dyes do not have a high diffusibility within the layer, the hydrophilic binder layer may be located between the intermediate layer and the base sheet or it may be located between the intermediate layer and the receiving layer. Here, whether or not a dye has a high diffusibility is determined by establishing the intermediate layer which does not contain hydrophilic binder as described above in an embodiment in which there is no hydrophilic binder layer and deciding whether or not the extent of fading of a transfer image (fading on ageing under conditions of 80° C. for 3 days or 60° C. for 1 week) is greater than that observed when no such layer has been established.

Intermediate layers which do not contain hydrophilic binders include either cushioning layers or porous layers, depending on the material from which they are constituted. Resins which are satisfactory under the conditions described above include, for example, polyurethane resins, polyester resins, polybutadiene resins, polyacrylic acid ester resins, epoxy resins, polyamide resins, rosin modified phenolic resins, terpene/phenol resins and ethylene/vinyl acetate copolymer resins.

One, or mixtures of two or more, of the above mentioned resins can be used.

The following methods may be used to form porous layers: (1) Methods in which a liquid consisting of an emulsion of a synthetic resin, such as polyurethane for example, or a synthetic rubber latex, such as a methyl methacrylate/butadiene based synthetic rubber emulsion, which has been agitated mechanically to incorporate bubbles is coated onto a base sheet and dried. (2) Methods in which a liquid obtained by mixing a foaming agent with the above mentioned synthetic resin emulsions or synthetic rubber latexes is coated onto the base sheet and dried. (3) Methods in which a liquid obtained by mixing a foaming agent with a vinyl chloride plastisol, a synthetic resin such as polyurethane or a synthetic rubber such as a styrene/butadiene based synthetic rubber is coated onto a base sheet and foamed by heating. (4) Methods in which a liquid mixture consisting of a solution obtained by dissolving a thermoplastic resin or a synthetic rubber in an organic solvent and an inorganic solvent (including those consisting principally of water) which is less volatile than the said organic solvent and compatible with the said organic solvent, and in which the thermoplastic resin or synthetic rubber is not soluble, is coated onto the base sheet and dried, whereupon a microporous layer is formed.

The intermediate layers which do not contain hydrophilic binder may be established on both sides in cases where receiving layers are present on both sides of the base sheet, or on just one side of the base sheet.

The thickness of an intermediate layer which does not contain hydrophilic binder is from 0.5 to 50  $\mu\text{m}$ , and most desirably from 2 to 20  $\mu\text{m}$ .

An anti-static agent can be included in the receiving layer on at least one side, or at the surface of the receiving layer, of a thermal transfer receiving sheet of this invention. Examples of anti-static agents include surfactants, for example cationic surfactants (quaternary ammonium salts, polyamine derivatives etc.), anionic surfactants (alkylsulfonates etc.), amphoteric type surfactants and non-ionic surfactants, and also metal oxides such as aluminum oxide and tin oxide etc. In structures in which a receiving layer is only established on one surface, an anti-static agent may also be used on the opposite surface to that on which the receiving layer is established.

The thermal transfer receiving sheets of this invention are used in combination with thermal transfer sheets.

A thermal transfer sheet has essentially, on a base sheet, a thermal transfer layer (dye donating layer) which contains a binder and dye which sublimes or becomes mobile on the application of heat. Thermal transfer sheets are obtained by preparing a coating solution in which the well known dyes which sublime or become mobile on the application of heat are dissolved or dispersed in an appropriate solvent and coating this liquid onto one side of a base sheet of the type well known for use in thermal transfer sheets at a rate such as to provide a dry film thickness of some 0.2 to 5  $\mu\text{m}$ , and preferably of from 0.4 to 2  $\mu\text{m}$ , and drying to form a thermal transfer layer.

Furthermore, anti-static layers as disclosed, for example, in EP 194106A and slip layers as disclosed, for example, in JP-A-62-51490 can be established, as required.

Dyes which are useful for forming thermal transfer layers of this type include all of those dyes which have

been used in thermal transfer sheets in the past, but the use of dyes of low molecular weight, i.e., 150 to 180, is especially desirable in this invention, and the dyes are selected in consideration of their transfer temperature, hue, light resistance and their solubility or diffusibility in inks and binder resins, etc.

In practical terms, examples of such dyes include disperse dyes, basic dyes and oil soluble dyes, and examples of actual dyes which can be used include "Sumicron Yellow E4GL", "Dyanics Yellow H2G-FS", "Miketone Polyether Yellow 3GSL", "Kayaset Yellow 937", "Sumicron Red EFB", "Dyanics Red ACE", "Miketone Polyether Red FB", "Kayaset Red 126", "Miketone Fast Brilliant Blue B", and "Kayaset Blue 136".

Furthermore, use can be made of the yellow dyes disclosed, for example, in JP-A-59-78895, JP-A-60-28451, JP-A-60-28453, JP-A-60-53564, JP-A-61-148096, JP-A-60-239290, JP-A-60-31565, JP-A-60-30393, JP-A-60-53565, JP-A-60-27954, JP-A-61-262191, JP-A-152563, JP-A-61-244595, JP-A-62-196186, JP-A-63-142062, JP-A-63-39380, JP-A-62-290583, JP-A-63-11094, JP-A-63-111095, JP-A-63-122954, JP-A-63-71392, JP-A-63-74685, JP-A-63-74688 and U.S. patent application Ser. No. 318,871 filed on Mar. 6, 1989 (dyes which can be represented by the general formula indicated below.



In this formula,  $R^1$  represents a hydrogen atom, an alkyl group, an alkoxy group, an aryl group, an alkoxy-carbonyl group, a cyano group or a carbamoyl group,  $R_2$  represents a hydrogen atom, an alkyl group or an aryl group,  $R_3$  represents an aryl group or a heterocyclic group, and  $R_4$  and  $R_5$  may be the same or different, each representing a hydrogen atom or an alkyl group. Moreover, the above mentioned substituent groups may be further substituted.)

Use can also be made of the magenta dyes disclosed, for example, in JP-A-60-223862, JP-A-60-28452, JP-A-60-31563, JP-A-59-78896, JP-A-60-31564, JP-A-60-303391, JP-A-61-227092, JP-A-61-227091, JP-A-60-30392, JP-A-60-30694, JP-A-60-131293, JP-A-61-227093, JP-A-60-159091, JP-A-61-262190, JP-A-62-33688, JP-A-63-5992, JP-A-61-12392, JP-A-62-55194, JP-A-62-297593, JP-A-63-74685, JP-A-63-74688, JP-A-62-97886, JP-A-62-132685, JP-A-61-163895, JP-A-62-211190, JP-A-62-99195 and GB-A-2209341 (dyes of the general formula indicated below).



In this formula,  $R_1$  and  $R_2$  represents hydrogen atoms, halogen atoms, alkyl groups, cycloalkyl groups, alkoxy groups, aryl groups, aryloxy groups, aralkyl groups, cyano groups, acylamino groups, sulfonylamino groups.

groups, alkoxycarbonyl groups, carbamoyl groups, sulfamoyl groups, sulfonyl groups, acyl groups or amino groups, and R<sub>3</sub> and R<sub>4</sub> represent alkyl groups, cycloalkyl groups, aralkyl groups or aryl groups. R<sub>3</sub> and R<sub>4</sub> may also be joined together to form a ring, and rings may also be formed by R<sub>2</sub> and R<sub>3</sub>, and by R<sub>2</sub> and R<sub>4</sub>. Moreover, n represents an integer of



value from 0 to 3. X, Y and Z represent T,0260 or nitrogen atoms. (Here, R<sup>5</sup> represents a hydrogen atom, an alkyl group, a cycloalkyl group, an aralkyl group, an aryl group, an alkoxy group, an aryloxy group or an amino group.) Furthermore, when X and Y or Y and Z are



they may be joined together to form saturated or unsaturated carbocyclic rings. The substituent groups indicated above may be further substituted.).

Use can also be made of the cyan dyes disclosed, for example, in JP-A-59-78894, JP-A-59-227490, 60-151098, JP-A-59-227493, JP-A-61-244594, JP-A-59-117948, JP-A-60-131292, JP-A-60-172591, JP-A-60-151097, JP-A-60-131294, JP-A-60-217-266, JP-A-60-31559, JP-A-60-53563, JP-A-61-255897, JP-A-60-239289, JP-A-61-22993, JP-A-61-19396, JP-A-61-368493, JP-A-61-35994, JP-A-61-31467, JP-A-61-148269, JP-A-61-49893, JP-A-61-57651, JP-A-60-23291, JP-A-60-239292, JP-A-61-284489, JP-A-62-191191, JP-A-62-138291, JP-A-62-288656, JP-A-63-57293, JP-A-63-15853, JP-A-63-144089, JP-A-63-15790, JP-A-62-311190, JP-A-63-74685, JP-A-63-74688, JP-A-62-132684, JP-A-62-87393, JP-A-62-255187 and U.S. patent application Ser. No. 218,789 filed on July 14, 1988 (dyes of the general formula indicated below.



In this formula, Q<sub>1</sub> represents a group of atoms, including at least one nitrogen atom, which is required to form, together with the carbon atoms to which they are bound, a nitrogen containing heterocyclic ring which incorporates at least five atoms, R<sub>1</sub> represents an acyl group or a sulfonyl group, R<sub>2</sub> represents a hydrogen atom or an aliphatic group which has from 1 to 6 carbon atoms, R<sub>3</sub> represents a hydrogen atom or a halogen atom, an alkoxy group or an aliphatic group which has from 1 to 6 carbon atoms, R<sub>4</sub> represents a halogen atom, an alkoxy group or an aliphatic group which has from 1 to 6 carbon atoms, and n represents an integer of value 0 to 4. R<sub>3</sub> may be joined to R<sub>1</sub> or R<sub>2</sub> or R<sub>4</sub> to form a ring. R<sub>5</sub> and R<sub>6</sub> represent hydrogen atoms, aliphatic groups which have from 1 to 6 carbon atoms, or aromatic groups. R<sub>5</sub> and R<sub>6</sub> may also be joined together to form

a ring. Furthermore, R<sub>5</sub> and/or R<sub>6</sub> may be joined with R<sub>4</sub> to form rings.).

Furthermore all of the well known binder resins used for this purpose in the past can be used as the binder resins which are used together with the dyes described above, and the binder resin is usually selected to provide a high resistance to heat and properties such that the migration of the dye is not impeded when it is heated. For example, use can be made of polyamide based resins, polyester based resins, epoxy based resins, polyurethane based resins, polyacrylic resins (for example, polymethyl methacrylate, polyacrylamide, polystyrene-2-acrylonitrile), vinyl based polymers, polyvinylpyrrolidone, polyvinyl chloride based resins (for example, vinyl chloride/vinyl acetate copolymers), polycarbonate based resins, polystyrene, polyphenylene oxide, cellulose based resins (for example, methylcellulose, ethylcellulose, carboxymethylcellulose, cellulose acetate hydrogen phthalate, cellulose acetate, cellulose acetate propionate, cellulose acetate butyrate, cellulose triacetate), polyvinyl alcohol based resins (for example, polyvinyl alcohol and partially saponified polyvinyl alcohol such as polyvinyl butyral, petroleum based resins, rosin derivatives, coumarone/indene resins, terpene based resins and polyolefin based resins (for example, polyethylene, polypropylene).

Binder resins of this type are preferably used at a rate, for example, of from about 80 to 600 parts by weight per 100 parts by weight of dye.

In this invention, the ink solvents known in the past can be used freely as ink solvents for the dissolution or dispersion of the above mentioned dyes and binder resins. Actual examples include alcohols such as methanol, ethanol, isopropyl alcohol, butanol and isobutanol, ketones such as methyl ethyl ketone, methyl isobutyl ketone and cyclohexanone, aromatic solvents such as toluene and xylene, halogenated solvents such as dichloromethane and trichloroethane, dioxane, and tetrahydrofuran, and mixtures of these solvents can also be used. These solvents must be selected and used in accordance with providing the prescribed concentration of the dye which is being used and providing for a satisfactory dissolution or dispersion of the binder resin. For example, the use of an amount of solvent about 9 to 20 times the total amount of dye and binder resin is desirable.

The thermal transfer sheets obtained in the way described above are contacted or laminated with the thermal transfer receiving sheets of this invention and heated in accordance with an image signal by means of a heating device such as a thermal head, for example, from either side, but preferably from the reverse side of the thermal transfer sheet. As a result of heating, the dye in the thermal transfer sheet can be moved and transferred in accordance with the magnitude of the thermal energy applied, simply and with comparatively low energy, to the thermal transfer receiving sheet, and it is possible to obtain color images which have excellent sharpness and resolution.

Any of base sheets known in the art can be used for the base sheet of the thermal transfer sheet which is used in this invention. For example, the base sheets may consist of polyester (for example polyethylene terephthalate), polyamide, polycarbonate, glassine paper, condenser paper, cellulose ester, fluoropolymer, polyether, polyacetal, polyolefin, polyimide, polyphenylene sulfide, polypropylene, polysulfone or cellophane.

The base sheet used for the thermal transfer sheet is generally of thickness from 2 to 30  $\mu\text{m}$ . The sheets may be covered with an under-layer, as required. Furthermore, the reverse side may be coated with a slipping layer in order to prevent the thermal head from sticking to the base sheet. Slipping layers of this type consist of lubricating substances, such as surfactants, liquid lubricants, solid lubricants or mixtures of these materials, and the layers may or may not contain a polymer binder.

Preferred embodiments of the invention are indicated below.

(a) Thermal transfer receiving sheets as disclosed in wherein the hydrophilic binder of the hydrophilic binder layer is gelatin.

(b) Thermal transfer receiving sheets wherein the coated weight of gelatin is from 0.4 to 3 g/m<sup>2</sup>.

(c) Thermal transfer receiving sheets wherein the base sheet is a polyolefin coated paper.

The invention is described in more detail below by means of illustrative examples.

### EXAMPLE 1

#### Preparation of the Thermal Transfer Sheet (A)

A polyester film (Lumirror, made by Toray Co., Ltd.) of thickness 4.5  $\mu\text{m}$  which had a heat resistant slip film consisting of thermoset acrylic resin established on one side was used as a base and thermal transfer receiving sheet (A) was obtained by coating a thermal transfer layer forming ink of which the composition is indicated below in such a way as to provide a coated weight after drying of 1 g/m<sup>2</sup> on the opposite surface of the base to that on which the heat resistant slip layer had been established.

#### Magenta Ink Composition for Thermal Transfer Layer

|                                                                                  |           |
|----------------------------------------------------------------------------------|-----------|
| Dispersed Dye (Disperse Red 60, MS Red G, made by Mitsui Toatsu Chemicals, Inc.) | 3.6 parts |
| Dispersed Dye (Disperse Violet 26, Macrolex Violet R, made by Bayer AG)          | 2.4 parts |
| Polyvinyl butyrate Resin (Eslec BX-I, made by Sekisui Chemicals Co, Ltd.)        | 4.3 parts |
| Methyl ethyl ketone                                                              | 45 parts  |
| Toluene                                                                          | 45 parts  |

#### Preparation of the Thermal Transfer Receiving Sheet

Low density polyethylene which had been milled with titanium oxide and ultramarine was laminated onto one side of a top quality paper as a base sheet and the other side was laminated with high density polyethylene. The low density polyethylene laminated side of this polyethylene coated paper was then coated with the hydrophilic binder layer composition (1) as shown in table 1.

| Hydrophilic Binder Layer Composition (1)                                                 |             |
|------------------------------------------------------------------------------------------|-------------|
| Gelatin                                                                                  | 60 grams    |
| Water                                                                                    | 3,000 grams |
| Surfactant                                                                               | 2.3 grams   |
| C <sub>4</sub> H <sub>9</sub> CH(C <sub>2</sub> H <sub>5</sub> )OCOCH <sub>2</sub>       |             |
| C <sub>4</sub> H <sub>9</sub> CH(C <sub>2</sub> H <sub>5</sub> )OCOCH—SO <sub>3</sub> Na |             |
| Viscosity increasing agent (Poly(potassium styrenesulfonate))                            | 1.4 grams   |

Moreover, the receiving Layer coating composition (2) of which the composition is indicated below was

coated by wire bar coating over the hydrophilic binder layer to provide a dry film thickness of 10  $\mu\text{m}$ , and the transfer receiving sheets (1) to (4) were obtained in this way.

Drying was accomplished by natural drying in a dry atmosphere followed by oven drying at 100° C. for a period of 30 minutes.

| Receiving Layer Coating Composition (2)                                              |          |  |
|--------------------------------------------------------------------------------------|----------|--|
| Polyester Resin (Vylon 280, made by Toyobo Co., Ltd.)                                | 14 grams |  |
| Isocyanate Based Curing Agent (KP-90, made by Dainippon Ink and Chemicals Co., Ltd.) | 3 grams  |  |
| Amino-modified Silicone Oil (KF-857, made by Shin-etsu Silicone Co., Ltd.)           | 0.5 gram |  |
| Epoxy-modified Silicone Oil (KF-100T, made by Shin-etsu Silicone Co., Ltd.)          | 0.5 gram |  |
| Triphenyl phosphate                                                                  | 6 grams  |  |
| Methyl ethyl ketone                                                                  | 85 ml    |  |
| Toluene                                                                              | 85 ml    |  |
| Cyclohexanone                                                                        | 30 ml    |  |

Moreover, the thermal transfer sheet and the thermal transfer receiving sheets obtained in the ways indicated above were laminated together in such a way that the thermal transfer layer was in contact with the receiving layer and printing was carried out using a thermal head from the support side of the thermal transfer sheet under conditions of a thermal head output 0.25 W/dot, a pulse width 0.2 to 15 msec, dot density 6 dots/mm, and the magenta dye dyed the receiving layer of the thermal transfer receiving layer.

Next, the thermal transfer receiving sheet was stored for 1 week in the dark at 80° C. and fading of the image in the dyed parts was investigated. Furthermore, the extent of curl of thermal transfer receiving sheets after aging for 5 hours under conditions of 25° C., 10% RH was also investigated. The results obtained are shown in Table 1.

Moreover, in Table 1, the evaluation of fading was made using three categories, namely A: Virtually no fading observed at all, B: Slight fading observed, and C: Pronounced fading.

The extent of curl was evaluated by the following manner. The receiving sheet having a dimension of 10 cm × 12 cm was placed on a flat plate in such a manner that the concave of the sheet was made upward. The extent of curl was evaluated by the distance between the corner of the receiving sheet and the surface of the flat plate. (+) means that the receiving layer was made downward, and (—) means that the receiving layer was made upward when the concave of the sheet was made upward.

TABLE 1

| Number of receiving sheet | Coated weight of hydrophilic binder layer composition (g/m <sup>2</sup> ) | Curl (mm) |           |
|---------------------------|---------------------------------------------------------------------------|-----------|-----------|
|                           |                                                                           | Fading    | Curl (mm) |
| 1 (Comparison)            | 0                                                                         | C         | -5        |
| 2 (Comparison)            | 0.05                                                                      | C         | -5        |
| 3 (Invention)             | 0.15                                                                      | B         | -5        |
| 4 (Invention)             | 0.3                                                                       | A         | -5        |
| 5 (Invention)             | 1.0                                                                       | A         | -4        |
| 6 (Invention)             | 1.5                                                                       | A         | -3        |
| 7 (Invention)             | 2.0                                                                       | A         | +3        |
| 8 (Invention)             | 3.0                                                                       | A         | +15       |
| 9 (Invention)             | 4.0                                                                       | A         | +28       |

TABLE 1-continued

| Number of receiving sheet | Coated weight of hydrophilic binder layer composition (g/m <sup>2</sup> ) | Fading | Curl (mm) |
|---------------------------|---------------------------------------------------------------------------|--------|-----------|
| 10 (Invention)            | 6.0                                                                       | A      | +35       |

It is clear from Table 1 that the thermal transfer receiving sheets of this invention exhibited little fading on ageing after image formation, and that they were not liable to curling when the coated weight is 3 g/m<sup>2</sup> or less.

### EXAMPLE 2

Thermal transfer receiving sheets 21 to 25 were prepared in the same way as the thermal transfer receiving sheets in Example 1 except that the hydrophilic binder layer composition (1) was replaced by the hydrophilic binder layer composition (3) indicated below, and the receiving layer coating composition (2) was replaced by the receiving layer coating composition (4) indicated below, and the thermal transfer receiving sheets were evaluated in the same way as in Example 1.

| Hydrophilic Binder Layer Composition (3)                                                                             |             |
|----------------------------------------------------------------------------------------------------------------------|-------------|
| Gelatin                                                                                                              | 60 grams    |
| Water                                                                                                                | 3,000 grams |
| Surfactant                                                                                                           | 2.3 grams   |
| C <sub>4</sub> H <sub>2</sub> CH(C <sub>2</sub> H <sub>5</sub> )OCOCH <sub>2</sub>                                   |             |
| C <sub>4</sub> H <sub>2</sub> CH(C <sub>2</sub> H <sub>5</sub> )OCOCH—SO <sub>3</sub> Na                             |             |
| Viscosity Increasing Agent (NH <sub>2</sub> CH=CHSO <sub>2</sub> CH <sub>2</sub> CONHCH <sub>2</sub> —) <sub>2</sub> | 1.8 grams   |

| Receiving Layer Coating Composition (4)                                              |          |
|--------------------------------------------------------------------------------------|----------|
| Polyester Resin (Vylon 300, made by Toyobo Co., Ltd.)                                | 20 grams |
| Isocyanate based Curing Agent (KP-90, made by Dainippon Ink and Chemicals Co., Ltd.) | 3 grams  |
| Amino-modified silicone Oil (KF-857, made by Shin-etsu Silicone Co., Ltd.)           | 0.5 gram |
| Epoxy-modified Silicone Oil (kf-100t, made by Shin-etsu Silicone Co., Ltd.)          | 0.5 gram |
| Methyl ethyl ketone                                                                  | 100 ml   |
| Toluene                                                                              | 100 ml   |

The results obtained are shown in Table 2.

TABLE 2

| Number of receiving sheet | Coated wt. of hydrophilic binder layer composition (g/m <sup>2</sup> ) | Fading | Curl |
|---------------------------|------------------------------------------------------------------------|--------|------|
| 21 (composition)          | 0                                                                      | C      | -5   |
| 22 (Invention)            | 0.3                                                                    | A      | -5   |
| 23 (Invention)            | 1                                                                      | A      | -3   |
| 24 (Invention)            | 3                                                                      | A      | +10  |
| 25 (Invention)            | 4                                                                      | A      | +24  |

It is clear from Table 2 that the thermal transfer receiving sheets of this invention exhibited little fading on ageing after image formation, and that they were not liable to curling. However, the curling properties clearly became poorer as the coated weight of hydrophilic binder layer was increased.

### EXAMPLE 3

Thermal transfer receiving sheets 31 to 34 were prepared in the same way as in Example 1 except that the

hydrophilic binder layer was modified to (5) indicated below, and the samples were evaluated in the same way as before.

| 5 |    | Hydrophilic Binder Layer Composition (5)                                                      |             |
|---|----|-----------------------------------------------------------------------------------------------|-------------|
|   |    | Hydrophilic Binder (see Table 3)                                                              | 60 grams    |
|   |    | Water                                                                                         | 3,000 grams |
|   | 10 | Surfactant C <sub>4</sub> H <sub>2</sub> CH(C <sub>2</sub> H <sub>5</sub> )OCOCH <sub>2</sub> | 2.3 grams   |
|   |    | C <sub>4</sub> H <sub>2</sub> CH(C <sub>2</sub> H <sub>5</sub> )OCOCH—SO <sub>3</sub> Na      |             |

The results obtained are shown in Table 3.

TABLE 3

| Number of receiving sheet | Hydrophilic binder     | Coated wt. (g/m <sup>2</sup> ) | Fading |
|---------------------------|------------------------|--------------------------------|--------|
| 31 (Comparison)           | None                   | 0                              | C      |
| 32 (Invention)            | Hydroxyethyl-cellulose | 1                              | B      |
| 33 (Invention)            | Polyacrylamide         | 1                              | B      |
| 34 (Invention)            | Poly(vinyl alcohol)    | 1                              | B-A    |

It is clear from Table 3 that the establishment of a hydrophilic binder layer provided an improvement in respect of image fading.

### EXAMPLE 4

Thermal transfer receiving sheets 41 to 43 were prepared in the same way except that synthetic paper (YUPO-FPG-150: Made by Oji Yuka K.K.) was used for the base sheet instead of the polyethylene coated paper used in Example 1, and the samples so obtained were evaluated in the same way as before. The results obtained are shown in Table 4.

TABLE 4

| Number of receiving sheet | Coated wt. of hydrophilic binder layer composition (g/m <sup>2</sup> ) | Fading |
|---------------------------|------------------------------------------------------------------------|--------|
| 41 (Comparison)           | 0                                                                      | C-B    |
| 42 (Invention)            | 0.1                                                                    | B      |
| 43 (Invention)            | 1                                                                      | A      |

It is clear that when synthetic paper is used, the establishment of a hydrophilic binder layer of this invention provides an improvement in respect of image fading. Moreover, with all of samples 14 to 17, concave deformation of the thermally printed parts occurred as a result of the heat applied during image formation.

### EXAMPLE 5

#### Preparation of the Thermal Transfer Receiving Sheet

In the gelatin solution (A) having the following composition, the organic solvent solution of the dye receiving polymer (B) was dispersed and emulsified by a homogenizer.

| Gelatin solution (A)                                   |       |  |
|--------------------------------------------------------|-------|--|
| Gelatin                                                | 2.3 g |  |
| 5%-aqueous solution of sodium dodecyl-benzenesulfonate | 20 ml |  |
| Water                                                  | 80 ml |  |

| Solution of the dye receiving polymer (B)                                          |       |
|------------------------------------------------------------------------------------|-------|
| Polyester resin<br>(Vylon 300, made by Toyobo Co., Ltd.)                           | 7.0 g |
| Carboxy-modified silicone oil<br>(X-22-3710, made by Shin-etsu Silicone, Co. Ltd.) | 0.7 g |
| Methyl ethyl ketone                                                                | 20 ml |
| Toluene                                                                            | 10 ml |
| Triphenylphosphate                                                                 | 1.5 g |

10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8895  
8900  
8905  
8910  
8915  
8920  
8925  
8930  
8935  
8940  
8945  
8950  
8955  
8960  
8965  
8970  
8975  
8980  
8985  
8990  
8995  
9000  
9005  
9010  
9015  
9020  
9025  
9030  
9035  
9040  
9045  
9050  
9055  
9060  
9065  
9070  
9075  
9080  
9085  
9090  
9095  
9100  
9105  
9110  
9115  
9120  
9125  
9130  
9135  
9140  
9145  
9150  
9155  
9160  
9165  
9170  
9175  
9180  
9185  
9190  
9195  
9200  
9205  
9210  
9215  
9220  
9225  
9230  
9235<br

TABLE 7-continued

| Number receiving sheet | Coated weight of hydrophilic binder layer composition (g/m <sup>2</sup> ) | Fading | Curl (mm) |
|------------------------|---------------------------------------------------------------------------|--------|-----------|
| 605 (Invention)        | 2.0                                                                       | A      | +1        |
| 606 (Invention)        | 4.0                                                                       | A      | +16       |
| 607 (Invention)        | 8.0                                                                       | A      | +31       |
| 608 (Invention)        | 16.0                                                                      | A      | +32       |

It is clear from the results in Table 7 that the thermal transfer receiving sheets of this invention exhibited little fading on aging after image formation. Particularly, when the coated amount of gelatin in the hydrophilic binder layer was 0.4 g/m<sup>2</sup> or more, the receiving sheets exhibited substantially no fading, while the extent of curl was increased when the coated amount of gelatin in the hydrophilic binder layer was 3 g/m<sup>2</sup> or more.

#### EXAMPLE 7

Thermal transfer receiving sheets 701 to 707 were prepared in the same manner as in the preparation of receiving sheets 501 to 507 except that the following receiving layer coating composition was used.

##### Receiving Layer Coating Composition

20 g of polyester resin (Vylon 290, made by Toyobo Co., Ltd.) and 2 g of diphenyl phthalate were dissolved in 30 ml of toluene and 70 ml of methyl ethyl ketone. The solution obtained was dispersed and emulsified in 100 ml of water containing 0.25 g of sodium dodecylbenzenesulfonate using a homogenizer at 15,000 rpm for 10 minutes. 5 cc of the solution of fluorine surface active agent used in Example 5 was added to the above emulsion to prepare the receiving layer coating composition.

The thermal transfer receiving sheets 701 to 707 were evaluated in the same manner as in Example 5. The results obtained are shown in Table 8 below.

TABLE 8

| Number receiving sheet | Coated weight of hydrophilic binder layer composition (g/m <sup>2</sup> ) | Fading | Curl (mm) |
|------------------------|---------------------------------------------------------------------------|--------|-----------|
| 701 (Comparison)       | 0                                                                         | C      | -5        |
| 702 (Invention)        | 0.1                                                                       | B      | -5        |
| 703 (Invention)        | 0.5                                                                       | A      | -4        |
| 704 (Invention)        | 1.0                                                                       | A      | -3        |
| 705 (Invention)        | 2.0                                                                       | A      | -2        |
| 706 (Invention)        | 4.0                                                                       | A      | +15       |
| 707 (Invention)        | 10.0                                                                      | A      | +35       |

It is clear from the results in Table 8 that the thermal transfer receiving sheets of this invention exhibited little fading on aging after image formation. Particularly, when the coated amount of gelatin in the hydrophilic binder layer was 0.4 g/m<sup>2</sup> or more, the receiving sheets exhibited substantially no fading, while the extent of curl was increased when the coated amount of gelatin in the hydrophilic binder layer was 3 g/m<sup>2</sup> or more.

While the invention has been described in detail and with reference to specific examples thereof, it will be apparent to one skilled in the art that various changes and modifications can be made therein without departing from the spirit and scope thereof.

What is claimed is:

1. A thermal transfer receiving sheet adapted to receiving a dye from a thermal transfer sheet containing a dye capable of being sublimed or rendered mobile by heat, wherein said thermal receiving sheet comprises at least one receiving layer for receiving dye provided on a base sheet, and said base sheet comprises a support having at least one hydrophilic binder provided on the support between the support and the receiving layer, wherein said hydrophilic binder is gelatin.
2. A thermal transfer receiving sheet as in claim 1, wherein the amount of said hydrophilic binder is from 0.4 to 3 g/m<sup>2</sup>.
3. A thermal transfer receiving sheet as in claim 1, wherein said base sheet is a polyethylene coated paper.

\* \* \* \* \*